

Jan. 23, 1934.

R. A. J. THENOZ

1,944,378

PROCESS AND APPARATUS FOR PRODUCING DULL LUSTER RAYON

Filed Jan. 24, 1930



Fig. 3.



Fig. 4.

Fig. 5.



Fig. 6.



Fig. 8.



Raymond A. J. Thenoz <sup>Inventor</sup>  
By Alexander Fawell <sup>Attorneys</sup>

## UNITED STATES PATENT OFFICE

1,944,378

PROCESS AND APPARATUS FOR PRODUC-  
ING DULL LUSTER RAYONRaymond Alfred Joseph Thenoz, Milan, Italy,  
assignor to Ruth-Aldo Company, Inc., a cor-  
poration of New YorkApplication January 24, 1930, Serial No. 423,166,  
and in Italy July 16, 1929

5 Claims. (Cl. 18—8)

This invention is a novel improvement in the production of so-called artificial silk commonly called rayon from cellulose esters such as cellulose acetate or cellulose nitrate. The object 5 of the invention is to produce a dull luster rayon and this is accomplished by so forming the filament that it will have more than two re-entrant reflective surfaces though it may vary in contour of its cross section at different portions of its 10 length. This result is obtained by my novel method of and apparatus for treating the filament during the spinning thereof. The invention includes a novel process for spinning such filament, novel apparatus for use in such operation, and 15 the novel product of such process.

One of the commercially objectionable properties of rayon as heretofore produced has been the high luster of the thread or fabric believed to be due to the reflection of light from the nearly 20 flat sides of the individual filaments which form the thread. Attempts to reduce the reflective properties of such high luster rayon have been made in various ways; for example, by introducing a pigment, by chemical after-treatment for 25 roughening the surface and in other ways.

I have discovered a novel method of and apparatus for producing a dull luster rayon which may readily be adapted for use in many factories 30 now equipped for making rayon yarn. To enable others to understand and use the invention I will describe the same with reference to the accompanying drawing, and then set forth in the 35 claims the essentials of the invention and the novel process, product and apparatus embraced within the invention.

In said drawing

Fig. 1 is a diagrammatic view of a typical heated spinning cell as used in the dry spinning process of manufacturing filaments from 40 solutions of cellulose esters in volatile solvents except that a fan has been added.

Fig. 2 is a greatly magnified view of a single orifice of the spinneret and a filament issuing 45 therefrom.

Figs. 3, 4, 5 and 6 are diagrammatic transverse sections of the filament as ordinarily produced respectively taken on the lines 3—3, 4—4, 5—5, and 6—6, in Fig. 2.

Fig. 7 is a greatly enlarged diagrammatic sectional elevation on the line 7—7 in Fig. 1 showing the high luster filaments produced by an ordinary cell operating under the old method.

Fig. 8 is a similar greatly magnified similar section on the line 7—7 in Fig. 1 illustrating the

dull luster filaments produced in accordance with my invention.

It is well known that certain forms of artificial silk, commonly known as rayon, are made by forcing a solution of cellulose nitrate, cellulose acetate, or other ester of cellulose, dissolved in a volatile solvent through very fine apertures in a spinneret and evaporating the solvent from the thus formed filaments by means of heated gases so that the filaments are eventually substantially freed from solvent and are hardened by such removal of the solvent. The gases employed may be atmospheric air or any suitable gaseous medium or mixtures thereof such as are commonly employed in the art—and I will hereinafter refer to them by the inclusive term gas or gases. A number of such filaments assembled together form a thread of rayon. For example a 20 or 25% solution of cellulose acetate dissolved in acetone can be used for the spinning 60 solution and fed to the spinneret and is ejected through the orifices of the spinneret as filaments and the acetone evaporated therefrom thus producing filaments of cellulose acetate.

I have discovered that by artificially producing 65 a shifting or movement of gases at an angle to the path of the jets adjacent the spinneret and before the filaments harden the cross section of the filament can be varied and rendered irregular and uneven in contour. This may be due to evaporation of the solvent from each jet issuing from the spinneret occurring unevenly on different 70 sides of the filament due to the differences in pressures thereon, or it may take place more rapidly 75 at the one side of the filament than from the other side, resulting in a different thickening of the cellulose ester film or skin formed on the exterior of the filament at the beginning of evaporation from the filament and consequently producing varying irregular cross sectional contours 80 of the filament.

Hitherto, the rule, desire, and purpose in the industry has been to evaporate the solvent from the filaments as uniformly as possible on all sides thereof, so that cross sections of the filament 85 would be alike throughout and alike in different filaments. The only exceptions have been on occasions when as an undesired violent air current has struck the filament in its semi-hardened state due to poor construction of the cell or when 90 some port in the cell has been opened causing an alteration in the composition of the gases therein or deflection of the filaments. In such 95 undesired exceptional and accidental cases and times the evaporation does not take place with 100 105 110

the desired uniformity and the filaments produced under such circumstances have been considered imperfect and undesirable.

I have discovered that by varying the lateral pressure of the gases on the filament during initial formation by imparting a movement to the gaseous atmosphere in a direction perpendicular, or inclined, to the length of the filament, and at a point adjacent the spinneret and before the filament has been solidified, I can produce such irregularities in the cross section of the filament that as a result, light, instead of being entirely reflected, is partly diffused and only partly reflected thereby, which effect is not obtainable with currents of gas travelling only parallel to the main movement of the filament and only in either the same or the opposite direction of movement of the filament.

The process may readily be carried on in a cell or chamber such as is commonly employed with a slight modification of or addition to such chamber as hereinafter explained.

A simple means for producing the desired current of gas is to place a small fan at the side of the spinning cell at a height just below the level of the spinneret. The concentration of the solvent in the gas about the spinneret will be changed but slightly if at all, because the fan merely forces or deflects a part of the gas in or passing through the cell laterally against the filament near the spinneret and may be said to cause a lateral air bump or curve in the air current normally traversing the cell in a direction parallel with the filaments but usually moving in a direction opposite thereto.

In the diagram Fig. 1, *a* indicates an ordinary spinning cell having double walls *b* through which hot water or steam or other source of heat circulates; *c* and *d* are the inlet and outlet, respectively, for the gas supplied to the cell and by which the volatile solvent in the filaments is evaporated; and *f* is the spinneret located in the cell and constructed and operated in the usual manner. Such cells are commonly provided with ports for cleaning the spinneret, and means to control the temperature, the circulation of gas and to recover the volatilized solvent, etc. all of which are well known in the art and therefore not described.

Figure 2 represents a diagrammatic greatly magnified view of one of the orifices *A* of the spinneret *f* of any suitable kind, from which the cellulose ester solution, known as "collodion", is issuing, and shows how the composition of the filament changes progressively as it leaves the spinneret. Figure 3 shows a cross section of the filament on the line 3—3, Figure 2, operated in the usual manner, such filament being first tubular and having an exterior film *e* of partially solidified cellulose ester with an unchanged solution of cellulose ester in its interior. As the solvent evaporates, the exterior film *e* thickens and the amount of collodion in the interior decreases, due to the evaporation. This results in a partial collapse of the tubular film *e* in the same manner as a light walled rubber tube collapses under a partial vacuum. This stage is indicated in Fig. 4, which represents a cross section on the line 4—4, Fig. 2. Further evaporation of the solvent in the filament produces further contraction, as indicated in Fig. 5, which represents a cross section on line 5—5 in Fig. 2. When the solvent is all substantially evaporated by the usual process the filament is a flattened ribbon whose cross section

is indicated in Fig. 6, which is a cross section on the line 6—6 in Fig. 2.

The aforesaid consecutive changes in cross section take place and give the final cross section *g* (Fig. 6) when evaporation of the solvent proceeds uniformly according to the old methods hitherto used in spinning rayon filaments.

Figure 7 illustrates greatly magnified typical cross sections of filaments obtained by operating the spinning cell as hereinbefore customarily used in the industry; while Fig. 8 illustrates greatly magnified cross sections of filaments produced in the same spinning cell operated and equipped in accordance with my invention.

In my invention a spinning cell is provided with means adjacent the spinneret for producing a lateral deflection of the gaseous current or a subsidiary internal lateral gas current within the main gas current in the cell at an angle to the filaments adjacent the spinneret so that the filaments issuing from the spinneret will be subjected to lateral gas currents—whereby they are caused to assume irregular shapes in cross section during the hardening thereof as indicated in Fig. 8. A very simple means (shown diagrammatically in Fig. 1) is a small rotary screw or fan *h*, placed in the interior of the spinning cell *a* adjacent and to one side of the spinneret *f* which fan can be operated by any suitable means so as to produce a current of gas or deflection of gases in a direction inclined to the collodion filaments issuing from the spinneret.

Such lateral current or deflection of gas will so affect the evaporation of the solvent from the filament during the formative and hardening steps that instead of contracting regularly and uniformly, as in Figs. 3—6 it will contract irregularly and will have irregular and re-entrant surfaces as indicated at *g*<sup>1</sup> in Figure 8, whereby the light is partially reflected but more largely diffused by such surfaces. Consequently the resulting filament and the yarn and fabrics produced from such filament do not have the high luster of ordinary rayon but instead have a dull luster which is so much desired in present day fabrics. The tensile strength of the dull luster filaments obtained by my invention is essentially the same as that of filaments produced by the old processes.

It is not considered that each filament will have one and the same type of cross section throughout its length. Instead any single filament may have various cross sections at different parts of its length, and probably no two filaments will be exactly alike in cross section, as indicated in Fig. 8.

In the claims the term gas is intended to include, not only atmospheric air, but also any gas, or mixture of gases, or of air and gases, or any one of these which will carry away solvent evaporated from the collodion.

The lateral deflection of the gaseous currents adjacent the spinneret does not disturb the equilibrium conditions of the cell, and it is not necessary to admit thereto or carry away therefrom any other gas than would be used in the ordinary spinning process, nor to affect the pressure or concentration of the solvent or gases used in spinning the filament.

In other words the invention is applicable to the ordinary spinning cell, and the temperatures, flow of gases to and from the cell, the gas employed in the cell, and the quality of the solutions employed in forming the filament can remain as ordinarily used, and the cell can be

operated under just the same conditions to produce my improved filament as it is operated to produce the ordinary filament provided only that suitable means are employed to produce the lateral deflection of the gaseous current or varying pressures against the filaments in the formative steps thereof; and while I have shown and described a fan in the cell as the means for producing such deflection of the current or unequal pressures the invention is not restricted to such means.

I claim:

1. A process of producing low luster rayon in which the filament while in plastic condition is subjected to the impact of a transverse current of gas at a velocity sufficient to produce a substantial permanent deformation of the contour of the filament.

2. A process of producing low luster rayon in which the filament immediately adjacent a spinneret is subjected to the impact of a transverse current of gas at a velocity sufficient to produce a substantial permanent deformation of the contour of the filament.

25

3. A process as set forth in claim 1 in which the current of gas impinges on the filament substantially at right angles thereto.

4. A process of producing low luster rayon by spinning in a closed cell containing a gas in which the solvent vaporizes, including the production within the cell of a current of said gas impinging transversely on the filament in a zone where said filament is in plastic condition, and at a velocity sufficient to produce a substantial permanent deformation of the contour of said filament.

80

5. In apparatus for dry spinning rayon filaments, a spinning cell of the closed type adapted to retain gas in which the solvent vaporizes, a spinneret adjacent an end of the cell, and rotary fan means within the cell for creating in said gas adjacent the spinneret a transverse current directed across the path of the filaments adjacent the spinneret at a velocity sufficient to produce a substantial permanent deformation in the 95 contour of the filaments.

85

RAYMOND ALFRED JOSEPH THENOZ.

100

30

105

35

110

40

115

45

120

50

125

55

130

60

135

65

140

70

145

75

150